

Patented Feb. 24, 1925.

1,527,576

# UNITED STATES PATENT OFFICE.

ISAAC M. SCOTT AND SAMUEL PEACOCK, OF WHEELING, WEST VIRGINIA, AND WILLIAM EARL ARMSTRONG, OF MARTINS FERRY, OHIO, ASSIGNORS TO WHEELING STEEL & IRON COMPANY, OF WHEELING, WEST VIRGINIA, A CORPORATION OF WEST VIRGINIA.

## PROCESS OF COATING CONDUCTING MATERIALS WITH TIN.

No Drawing.

Application filed February 19, 1923. Serial No. 620,009.

To all whom it may concern:

Be it known that we, ISAAC M. SCOTT, SAMUEL PEACOCK, and WILLIAM EARL ARMSTRONG, all citizens of the United States, the said ISAAC M. SCOTT and SAMUEL PEACOCK residing at Wheeling, in the county of Ohio and State of West Virginia, and the said WILLIAM EARL ARMSTRONG residing at Martins Ferry, in the county of Belmont 10 and State of Ohio, have invented certain new and useful Improvements in Processes of Coating Conducting Materials with Tin; and we do hereby declare the following to be a full, clear, and exact description of the 15 invention, such as will enable others skilled in the art to which it appertains to make and use the same.

This invention relates to improvements in electro-tinning and more particularly to the 20 solution or electrolyte, and to a process whereby said electro-tinning can be carried out on a commercial scale and in a manner more economical than has been heretofore attained.

25 With these and other objects in view the invention consists in the novel steps and combinations of steps constituting the process, all as will be more fully hereinafter disclosed and particularly pointed out in the 30 claims.

In order that the precise invention may be the more clearly understood it is said:— In the electro-deposition of tin, great difficulty has been heretofore experienced in producing a dense and coherent deposit. This is especially emphasized when the objects to be electro-tinned are constructed of metals higher in the electro chemical series than is tin, such for example, as steel or iron. 40 Heretofore, articles constructed of metals, such as iron, were first electro-plated with a metal lower in the electro chemical series such for example as copper, and upon this last named metal the tin was deposited. But, solutions that are available for depositing the tin directly on iron or steel deteriorate rapidly, and cannot be operated on a commercial scale, economically, unless associated with a suitable restoring solution. These difficulties are all well known in this art.

On the other hand, this invention involves a solution and a method by which electro-

tinning can be carried out without difficulty and much more efficiently than heretofore; and this solution can be used for plating directly on steel and other metals higher in the electro chemical series. Further this method may be used for large scale operations with different concentrations and without causing a formation of colloidal or spongy deposits as in the prior procedures. The solutions contain a lower percentage of tin than those heretofore employed, they do not deteriorate or hydrolize to an objectionable extent, and they operate with almost 100% efficiency. This bath does not require a periodical addition of tin salts as heretofore, or in other words it is self sustaining.

It will be understood by those skilled in the art that the thickness of deposit or amount of tin plated per unit of surface will depend upon the length of time and the number of amperes used, irrespective of the voltage, but of course, the lower the voltage employed the more economical will be the deposition.

It has been found in practice that with say  $\frac{3}{4}$  to  $1\frac{1}{4}$  volts, good deposits are obtained with this solution.

In carrying out the invention in its preferred form, one may take, for example 3 parts by weight of a 50% commercial hydrofluoric acid (HF) and dissolve therein 1.6 85 parts by weight of boric acid  $H_3BO_3$ . These acids react with an evolution of heat and form an acid known as fluoboric acid or borofluohydric acid, the simplest formula of which is  $HBF_4$ . In this acid, one dissolves stannous oxide  $SnO$  until the acid has taken up the equivalent of 1.35 parts by weight of metallic tin, leaving about 31% of the acid present in the free state.

By this means there is produced a solution of stannous fluoborate  $Sn(BF_4)_2$  containing an excess of free fluoboric acid  $HBF_4$ . To increase the conductivity of this solution one adds a metallic salt of a metal higher in the electro-chemical series than iron, and prefers for this purpose the addition of 1.3 parts by weight of aluminum sulphate  $Al_2(SO_4)_3$  or 1.3 parts by weight of magnesium sulphate  $MgSO_4$ . This solution is then diluted with water to such a concentration that it will contain about  $1\frac{1}{3}$  ounces

of metallic tin to one gallon. In this diluted solution there is suspended metallic tin as an anode on a positive bus bar, and one suspends the articles to be plated such as sheet steel, in the solution and connects them to the negative bus bar whereby on the passage of a suitable electric current, the steel articles become plated with metallic tin.

10 It has been found it is also desirable to add so-called addition agents or brightening agents, such as molasses, gelatine, etc., to the solution for the purpose of obtaining somewhat improved and bright deposits. It is 15 preferred to use ordinary glue for this purpose and in a quantity of about .03 ounce per gallon of solution, but a larger amount will not interfere with the success of the process.

20 Instead of using stannous oxide  $\text{SnO}$  for introducing the tin into this solution, one may add other tin salts, such as stannous hydrate  $\text{Sn}(\text{OH})_2$ , or may dissolve in the solution metallic tin with or without the aid 25 of the electric current. It has been found that the economical addition of tin may also be obtained by suspending metallic tin as anodes in the solution, connected with a positive bus bar and suspending metal strips, 30 surrounded by porous cups in the solution, the metal strips being connected to a negative bus bar. By the passage of a suitable electric current, such as that above disclosed, the tin is dissolved from the anodes into the 35 solution and being unable to pass into the porous cups, it is taken up by the acid. When sufficient tin has been dissolved the cups are removed and the plating continued.

In the foregoing description there is disclosed a tin solution in a somewhat diluted form with an acid reaction, but the solution can be used in more concentrated forms such for example as in those having a plurality of times the concentration of that above mentioned. The solution can also be used in the neutral state and for certain purposes one prefers a neutral solution, for such last named solution is especially desirable when chemically pure tin is being deposited.

50 The above solution has proved satisfactory for the deposition of tin on various metals such as iron, steel and copper, and therefore, it is not desired to be limited to the procedure set forth in the description. This 55 solution and process may also be used with various modifications for numerous purposes that will readily suggest themselves to those skilled in the art without departing from the spirit of my invention.

For example, a conducting metal salt, carbon or other electric conductor may be deposited by well known means in the pores of a fabric or other material and tin may be deposited thereon by following the foregoing procedure. Therefore, it is not desired to be limited to the above disclosure except as may be required by the claims.

In our co-pending application Serial No. 620,010, filed February 19, 1923, for "electro-plating baths", a bath suitable for carrying out this process is disclosed and claimed.

What is claimed is:—

1. The process of coating tin on electric conductors which consists in providing an electrolytic solution containing tin dissolved in boro-fluohydric acid; immersing the article to be coated in said solution; and passing a current of electricity from said solution to said article to obtain the desired coating.

2. The process of coating tin on an electric conductor which consists in providing an electrolytic solution containing stannous fluoborate and a salt of a metal more electro-positive than iron; immersing the article to be coated in said solution as a cathode; and passing a current through said solution to said cathode to obtain the desired coating.

3. The process of coating iron or steel with tin which consists in providing a bath consisting essentially of stannous fluoborate; immersing the iron or steel article to be coated in said bath and making the same a cathode in an electrolytic circuit; and passing a current to obtain the desired coating.

4. The process of coating iron or steel with tin which consists in providing a bath consisting essentially of stannous fluoborate admixed with free boro-fluohydric acid; immersing the iron or steel article to be coated in said bath and making the same a cathode in an electrolytic circuit; and passing a current to obtain the desired coating.

5. The process of coating iron or steel with tin which consists in providing a bath consisting essentially of stannous fluoborate admixed with a substantial quantity of boro-fluohydric acid and a salt of a metal more electro-positive than iron; immersing the iron or steel article to be coated in said bath and making the same a cathode in an electrolytic circuit; and passing a current to obtain the desired coating.

In testimony whereof we affix our signatures.

ISAAC M. SCOTT.

SAMUEL PEACOCK.

WILLIAM EARL ARMSTRONG.